

## UNITED STATES PATENT OFFICE

2,340,920

## STABILIZED WHITE OIL

Francis M. Archibald, Elizabeth, N. J., and Carl A. Harris, Philadelphia, Pa., assignors to Standard Oil Development Company, a corporation of Delaware

No Drawing. Application August 12, 1942,  
Serial No. 454,550

4 Claims. (Cl. 252—52)

This invention relates to stabilized highly refined hydrocarbon oils of light lubricating oil consistency commonly termed white oils, particular grades of which are employed as medicinal oils. This application is a continuation-in-part of our co-pending application, Serial No. 293,950, filed September 8, 1939, which has matured into Patent 2,311,505 on February 16, 1943.

The hydrocarbon base oils of the compositions prepared according to the invention are obtained by highly refining petroleum distillates of light lubricating oil consistency by means of treatment with successive volumes of fuming sulfuric acid followed by neutralization, washing and generally percolating or contacting with clay. The oils refined in this manner have colors of at least 30+ Saybolt. They consist largely of paraffin and naphthene hydrocarbons and they have viscosities of above about 32 Saybolt-Universal seconds at 100° F. and preferably between about 55 and 350 seconds Saybolt Universal at 100° F. The oils so prepared are suitable as medicinal oils and are refined so as to pass the specifications for petrolatum liquidum U. S. P.

These highly refined oils are usually somewhat chemically unstable. Oftentimes the oils develop objectionable odors and tastes. Also, such highly treated oils upon exposure at elevated temperatures to metals, such as copper, cause staining of the metal. These effects appear to be connected with and are due presumably to the presence of unstable sulfur compounds formed by the interaction of concentrated sulfuric acid and certain organic compounds in the oils, particularly in those oils of Mid-Continent and Gulf Coast origins. These organic compounds are apparently present in traces and may also be introduced by contamination during handling the distillate in refineries making fuel oil and other low grade products. A test known as the copper strip test devised to indicate such instability is that of maintaining the oil at about 210° F. for about 2 hours in the presence of a highly polished copper strip; any tarnishing or discoloration is considered as evidence of instability. The presence of sulfur is readily demonstrated by removing the copper stain with nitric acid and testing for sulfates with barium chloride.

It was disclosed in our co-pending application, Serial No. 293,950, that the non-volatile, oil-soluble, relatively water insoluble, organic compounds of acidic characteristics and of molecular weight above about 120 may be added to these highly refined oils to combat the chemical instability. It was found that these compounds were satis-

factory addition agents to white oils in that they have suitable oil solubility and they do not impart a detectable taste to the composites in the concentrations in which they are used. Also, the compounds employed are relatively inexpensive and are added to the oils in very low concentrations. The present invention is an extension of the use of certain compounds of this class, namely, the mono-hydroxy aromatic carboxylic acids.

5 These compounds are particularly effective as stabilizing agents for mineral white oils difficult to correct by other compounds added as inhibitors or even by reprocessing in one form or another.

10 It has now been found that all mineral white oils are not equally responsive to correction of their instability characteristics by the addition of the inhibitory compounds disclosed in our co-pending application, Serial No. 293,950. It was stated in that prior application that one of the 15 tests to which finished oils are subjected is the hot acid test as described in the U. S. Pharmacopoeia (9th edition, page 315). In this test the finished oil resists the action of hot concentrated acid as shown by shaking together equal quantities of the oil and 95% sulfuric acid at 100° C. The acid from this test usually takes on color due to a slight reaction; if the color is no darker than a light amber the oil is said to pass the test. In the refining of stocks to produce white oils, 20 the improvement in the hot acid test follows the amount of acid employed up to a certain point and then further quantities of acid have decreasing refining effects and finally there is no improvement. Normally the hot acid test is employed as a control to indicate sufficiency of treatment.

25 It has been known for some time that there are some so-called technical white oils, i. e., oils of 30+ Saybolt but of low hot acid test which 30 do not pass the copper test and which are not made to pass the copper test by the addition of the inhibitor compounds commonly employed in white oil manufacture. It has now been found that when these technical white oils are given a further treatment with concentrated sulfuric acid and resultant products finished to give a U. S. P. hot acid test, then the instabilities of such added treated oils are readily corrected by the addition of from 0.01% to 0.00005% of a monohydroxy aromatic carboxylic acid. These compounds may be added directly to the oil or dissolved in a small amount of oil to make a concentrate, which is employed for blending into the oil.

35 Of the monohydroxy aromatic carboxylic acids suitable as inhibitors in white oils, it has been

found particularly advantageous to employ salicylic acid or the alkylated salicylic acids. These alkylated salicylic acids are more soluble in oil than salicylic acid itself and, therefore, blend much more readily and easily with the oil. The salicylic acids as a group are also colorless and free from odor and do not impart color or thermal instability in the mineral oil composites. Worthy of particular mention among the salicylic acids as being effective in concentrations of from 0.00005% to 0.01% of concentration are the following compounds and their respective solubilities in 100 grams of 55 Saybolt Viscosity at 100° F. mineral white oil:

|                                                  | Grams |
|--------------------------------------------------|-------|
| Salicylic acid                                   | .0328 |
| Tertiary butyl salicylic acid                    | .532  |
| Tertiary amyl                                    | .82   |
| Thymotic acid (methyl, isopropyl salicylic acid) | 1.105 |

It would seem that the monohydroxy aromatic carboxylic acids are unique as corrective agents for oils which cannot be suitably refined in any other manner. Thus purification of the oil is generally considered not advantageous because such processing is expensive and generally uncertain as to its sufficiency. Also, the oils improved by the compounds of this invention cannot be satisfactorily corrected by the addition of other types of inhibitors, such as oxidation or light stabilizing compounds. In this latter connection it was found that the meta and para benzoic acids had some effect as corrective agents in these oils but they were only about  $\frac{1}{10}$  as effective as salicylic acid. Beta resorcylic acid (di-hydroxy benzoic acid) and gallic acid (trihydroxy benzoic acid) were found to have little or no effect on the copper test. The effects of the various compounds in mineral oils of 90 Viscosity Saybolt at 100° F. containing the various compounds when subjected to the copper test are shown in the following tabulation:

|                      | Amount added | Copper test |            |
|----------------------|--------------|-------------|------------|
|                      |              | Percent     |            |
| Unblended oil        |              |             | Not. pass. |
| Salicylic:           |              |             |            |
| (O-hydroxy benzoic)  | .0001        | Pass.       |            |
| M-hydroxy benzoic    | .0001        | Not pass.   |            |
| M-hydroxy benzoic    | .001         | Pass.       |            |
| P-hydroxy benzoic    | .0001        | Not pass.   |            |
| P-hydroxy benzoic    | .001         | Pass.       |            |
| Beta resorcylic acid |              |             |            |
| Do.                  | .001         | Not pass.   |            |
| Do.                  | .01          | Do.         |            |
| Do.                  | .001         | Do.         |            |
| Do.                  | .01          | Do.         |            |

The particular effectiveness of the monohy-

droxy aromatic carboxylic acids as inhibitors in finished oils which have been treated with sufficient fuming sulphuric acid to pass the U. S. P. hot acid test by a practical margin appears connected with the removal, modification or stabilization of the unstable sulfur compounds previously produced in the oil as a result of the treatment with sulfuric acid of certain stocks. This opinion is supported by the observation that the staining which the inhibited oils cause upon copper strip at 210° F. is usually due to the formation of copper sulfide. No definite reason can be advanced for the formation of such unstable sulfur compounds in some stocks and the lack of formation of such compounds in other cases. The higher grade of paraffinic stock for example show little tendency to the formation of these compounds but they may be present in these oils as a result of contamination in their handling through pipe lines and tankage. Mid-Continent and Coastal base stocks on the other hand often show the instability and it would appear in these cases that it is connected with impurities in the base stock or formed during distillation, and then subsequently reactive with sulfuric acid during the final refining stages.

The invention is not to be limited to the use of the particular compounds shown nor to any theory with regard to the activity of the ingredients but only to the following claims in which it is desired to claim all the novelty inherent in the invention.

What is claimed is:

1. The method of stabilizing highly refined mineral white oils which comprises incorporating in a highly refined mineral white oil distillate which has been treated with sulfuric acid in an amount in excess of that required to be of U. S. P. mineral white oil quality, has a viscosity above about 32 Saybolt-Universal seconds at 100° F. and has a color of at least 30+ Saybolt, a monohydroxy aromatic carboxylic acid in an amount between 0.01% and 0.00005%.

2. The method of stabilizing highly refined mineral white oil according to claim 1 in which the said white mineral oil has a viscosity between about 55 and 350 Saybolt-Universal seconds at 100° F.

3. The method of stabilizing highly refined mineral white oil according to claim 1 in which the monohydroxy aromatic carboxylic acid is a salicylic acid.

4. The method of stabilizing highly refined mineral white oil according to claim 1 in which the monohydroxy aromatic carboxylic acid is an alkylated salicylic acid.

FRANCIS M. ARCHIBALD.  
CARL A. HARRIS.